

# United States Patent [19]

Malec

[11] 4,198,931

[45] Apr. 22, 1980

## [54] DIESEL FUEL

[75] Inventor: Robert E. Malec, Birmingham, Mich.

[73] Assignee: Ethyl Corporation, Richmond, Va.

[21] Appl. No.: 8,752

[22] Filed: Feb. 1, 1979

[51] Int. Cl.<sup>2</sup> ..... C10L 1/18; C10L 1/22

[52] U.S. Cl. ..... 123/1 A; 44/53;  
44/56; 44/57; 44/71; 123/198 A

[58] Field of Search ..... 44/53, 57, 71, 56;  
123/1 A, 198 A

## [56] References Cited

### U.S. PATENT DOCUMENTS

3,328,138 6/1967 Malec et al. ..... 44/71  
4,002,437 1/1977 Broeclx et ..... 44/66

### FOREIGN PATENT DOCUMENTS

2701588 7/1978 Fed. Rep. of Germany ..... 44/53

## OTHER PUBLICATIONS

English Translation of Brazilian Patent Application No.  
P17700392.

*Primary Examiner*—Winston A. Douglas

*Assistant Examiner*—J. V. Howard

*Attorney, Agent, or Firm*—Donald L. Johnson; Robert  
A. Linn; Willard G. Montgomery

## [57] ABSTRACT

An anti-wear compression ignition fuel for use in diesel  
engines comprising (1) a monohydroxy alkanol having  
from 1 to 5 carbon atoms, and (2) a wear inhibiting  
amount of an N-hydroxy hydrocarbonamide, e.g. N-  
hydroxy oleamide. Optionally, said fuel composition  
may also contain an ignition accelerator such as an  
organic nitrate.

41 Claims, No Drawings

## DIESEL FUEL

It has recently been disclosed in Brazilian patent application No. P 17700392 that alcohols, such as methanol and ethanol, can be substituted for conventional petroleum derived diesel fuels for burning in diesel engines, when used in combination with an ignition accelerator, such as ethyl nitrate or nitrite. Reportedly, the addition of alkyl nitrate or nitrite accelerators to the alcohol achieves a level of auto-ignition sufficient to operate in diesel engines. Unfortunately, these fuel compositions, devoid of any petroleum derived products, are notably deficient in lubricity or lubricating properties with the result that engine wear from the use of these fuels in internal combustion reciprocating diesel engines is a serious problem. Of particular concern are wear problems associated with the fuel injector mechanisms used in such engines. Wear problems have also been encountered in diesel engines operating on light diesel fuel oils as disclosed in U.S. Pat. No. 4,002,437.

The present invention relates to the use of certain hydroxamic acids to reduce the wear properties of diesel fuel compositions of the alcohol or alcohol containing type. U.S. Pat. No. 3,328,138 discloses gasoline containing hydroxamic acid as carburetor detergents.

## SUMMARY OF THE INVENTION

It has now been found that the addition of certain N-hydroxy hydrocarbonamides, also known as hydroxamic acids, to fuels adapted for use in diesel engines comprising a monohydroxy alkanol having from 1 to 5 carbon atoms and optionally containing an ignition accelerator such as an organic nitrate can significantly improve the wear characteristics of said fuels.

## DESCRIPTION OF THE PREFERRED EMBODIMENTS

A preferred embodiment of the present invention is an anti-wear compression ignition fuel for use in diesel engines comprising (1) a monohydroxy alkanol having from 1 to 5 carbon atoms, and (2) a wear inhibiting amount of an N-hydroxy hydrocarbonamide having the formula



wherein R is a hydrocarbon group having a valence of n and containing from 6 to about 51 carbon atoms and n is an integer from 1 to 3.

Another embodiment of the present invention is an anti-wear compression ignition fuel for use in diesel engines comprising (1) a monohydroxy alcohol having from 1 to 5 carbon atoms, (2) an ignition accelerator, and (3) a wear inhibiting amount of an N-hydroxy hydrocarbonamide having the formula



wherein R is a hydrocarbon group having a valence of n and containing from 6 to about 51 carbon atoms and n is an integer from 1 to 3.

A further embodiment of the present invention is a method for inhibiting engine wear in an internal combustion reciprocating diesel engine operating on a compression ignition fuel comprising (1) a monohydroxy alkanol having from 1 to 5 carbon atoms, (2) an ignition

accelerator, and (3) a wear inhibiting amount of an N-hydroxy hydrocarbonamide having the formula



wherein R is a hydrocarbon group having a valence of n and containing from 6 to about 51 carbon atoms and n is an integer from 1 to 3, said method comprising (a) supplying to the fuel induction system of said engine 10 said compression ignition fuel, (b) inducting air into the combustion chambers of said engine, (c) compressing said air, (b) injecting said compression ignition fuel into said combustion chambers containing said compressed air, (e) igniting said compressed mixture, and (f) exhausting the resultant combustion products resulting in reduced engine wear in said engine.

A still further embodiment of the present invention is a method for preparing a compression ignition fuel adapted for use in diesel engines having anti-wear properties which comprises blending (1) a wear inhibiting amount of an N-hydroxy hydrocarbonamide having the formula



wherein R is a hydrocarbon group having a valence of n and containing from 6 to about 51 carbon atoms and n is an integer from 1 to 3 with (2) a monohydroxy alkanol having from 1 to 5 carbon atoms, and (3) an ignition 25 accelerator.

Monohydroxy alcohols which can be used in the present invention include those containing from 1 to 5 carbon atoms. Preferred alcohols are saturated aliphatic monohydric alcohols having from 1 to 5 carbon atoms. Methanol, ethanol, propanol, n-butanol, isobutanol, amyl alcohol and isoamyl alcohol are preferred alcohols for use in the present invention. Of these, ethanol is the most preferred.

The N-hydroxy hydrocarbonamide component of the fuel composition of the present invention can be represented by the formula



wherein R is a hydrocarbon group having a valence of n and containing from 6 to about 51 carbon atoms and n is an integer from 1 to 3.

Representative N-hydroxy hydrocarbonamides are:

N-hydroxy hexanamide  
N-hydroxy heptanamide  
N-hydroxy octanamide  
N-hydroxy decanamide  
N-hydroxy dodecanamide  
N-hydroxy tetradecanamide  
N-hydroxy hexadecanamide  
N-hydroxy octadecanamide  
N-hydroxy eicosanamide  
N-hydroxy triacontanamide  
N-hydroxy oleamide  
N-hydroxy linoleamide  
N-hydroxy linoleamide dimer  
N-hydroxy linoleamide trimer

The latter two additives are the N-hydroxyamide of linoleic dimer and trimer. These usually occur in mixtures.

The most preferred additive is N-hydroxy oleamide.

The N-hydroxy hydrocarbonamides can be made by conventional methods. For example, Berichte, 1898, 31,

2191, discloses the preparation of a hydroxamic acid (now named N-hydroxyamide) by the reaction of a fatty acid ester with hydroxylamine. Suitable wear agents can be made in this manner starting with lower alkyl esters of fatty acids or mixtures of fatty acids (e.g. tall oil fatty acid esters, oleic acid esters, dimers and trimers of linoleic acid esters and the like).

Optionally, the fuel composition of the present invention may contain an ignition accelerator. The ignition accelerator component of the anti-wear compression ignition fuel composition of the present invention is preferably an organic nitrate. Preferred organic nitrates are substituted or unsubstituted alkyl or cycloalkyl nitrates having up to about 10 carbon atoms, preferably from 2 to 10 carbon atoms. The alkyl group may be either linear or branched. Specific examples of nitrate compounds suitable for use in the present invention include, but are not limited to the following:

methyl nitrate  
 ethyl nitrate  
 n-propyl nitrate  
 isopropyl nitrate  
 allyl nitrate  
 n-butyl nitrate  
 isobutyl nitrate  
 sec-butyl nitrate  
 tert-butyl nitrate  
 n-amyl nitrate  
 isoamyl nitrate  
 2-amyl nitrate  
 3-amyl nitrate  
 tert-amyl nitrate  
 n-hexyl nitrate  
 2-ethylhexyl nitrate  
 n-heptyl nitrate  
 sec-heptyl nitrate  
 n-octyl nitrate  
 sec-octyl nitrate  
 n-nonyl nitrate  
 n-decyl nitrate  
 n-dodecyl nitrate  
 cyclopentyl nitrate  
 cyclohexyl nitrate  
 methylcyclohexyl nitrate  
 isopropylcyclohexyl nitrate

and the esters of alkoxy substituted aliphatic alcohols, such as 1-methoxypropyl-2-nitrate, 1-ethoxypropyl-2-nitrate, 1-isoproxybutyl nitrate, 1-ethoxybutyl nitrate and the like. Preferred alkyl nitrates are ethyl nitrate, propyl nitrate, amyl nitrates and hexyl nitrates. Other preferred alkyl nitrates are mixtures of primary amyl nitrates or primary hexyl nitrates. By primary is meant that the nitrate functional group is attached to a carbon atom which is attached to two hydrogen atoms. Examples of primary hexyl nitrates would be n-hexyl nitrate, 2-ethylhexyl nitrate, 4-methyl-n-pentyl nitrate and the like. Preparation of the nitrate esters may be accomplished by any of the commonly used methods: such as, for example, esterification of the appropriate alcohol, or reaction of a suitable alkyl halide with silver nitrate.

Other conventional ignition accelerators may also be used in the present invention, such as hydrogen peroxide, benzoyl peroxide, etc. Further certain inorganic and organic chlorides and bromides, such as, for example, aluminum chloride, ethyl chloride or bromide may find use in the present invention as primers when used in

combination with the alkyl nitrate accelerators of the present invention.

The amount of N-hydroxy hydrocarbonamide used in the compression ignition fuel compositions of the present invention should be enough to provide the desired wear protection. This concentration is conveniently expressed in terms of weight percent of N-hydroxy hydrocarbonamide based on the total weight of the compression ignition fuel composition. A preferred concentration is from about 0.01 to about 2.0 weight percent. A more preferred range is from about 0.1 to about 1.0 weight percent.

The amount of alkyl nitrate or nitrite ignition accelerator used should be an amount which will achieve a level of auto-ignition sufficient to allow the operation of diesel engines on the fuel composition of the present invention. A useful range is from about 0.1 weight percent to about 10 weight percent based on the total weight of the compression ignition fuel composition.

Preferred amounts are between 0.5 weight percent to 5.0 weight percent.

Other additives may be used in formulating the compression ignition fuel compositions of the present inventions. These compounds include demulsifying agents, corrosion inhibitors, antioxidants, dyes, and the like, provided they do not adversely effect the anti-wear effectiveness of the N-hydroxy hydrocarbonamide.

Conventional blending equipment and techniques may be used in preparing the fuel composition of the present invention. In general, a homogeneous blend of the foregoing active components is achieved by merely blending the N-hydroxy hydrocarbonamide component of the present invention with the monohydroxy alkanol and, if desired, ignition accelerator component of the present invention in a determined proportion sufficient to reduce the wear tendencies of the fuel. This is normally carried out at ambient temperature. The following examples illustrate the preparation of some typical fuel compositions of the present invention.

40

#### EXAMPLE I

To a blending vessel is added 1000 parts of 190 proof ethanol and 20 parts of an N-hydroxy hydrocarbonamide. The mixture is stirred at room temperature until homogeneous forming a fuel composition useful for reducing and/or inhibiting the amount of engine wear in internal combustion reciprocating diesel engines operating on said fuel composition.

#### EXAMPLE II

To a blending vessel is added 1000 parts of 190 proof ethanol, and 1 part of an N-hydroxy hydrocarbonamide. The mixture is stirred at room temperature until homogeneous forming a fuel composition useful for reducing and/or inhibiting the amount of engine wear in internal combustion reciprocating diesel engines operating on said fuel composition.

The amounts of each ingredient in the foregoing compositions can be varied within the limits aforesdiscussed to provide the optimum degree of each property.

The lubricity or wear properties of the fuel compositions were determined in the 4-Ball Wear Test. This test is conducted in a device comprising four steel balls, three of which are in contact with each other in one plane in a fixed triangular position in a reservoir containing the test sample. The fourth ball is above and in contact with the other three. In conducting the test, the upper ball is rotated while it is pressed against the other

50

55

60

65

three balls while pressure is applied by weight and lever arms. The diameter of the scar on the three lower balls are measured by means of a low power microscope, and the average diameter measured in two directions on each of the three lower balls is taken as a measure of the anti-wear characteristics of the fuel. A larger scar diameter means more wear. The balls were immersed in base fuel containing the test additives. Applied load was 5 kg and rotation was at 1,800 rpm for 30 minutes at ambient temperature. Tests were conducted both with base fuel\* alone and base fuel containing the test additives. Results are as follows:

| Additive <sup>(1)</sup><br>Conc.<br>(wt. %) | Scar Diameter<br>(mm) |       |
|---------------------------------------------|-----------------------|-------|
|                                             | Run 1                 | Run 2 |
| None                                        | 0.89                  | 0.90  |
| 1.0                                         | 0.44                  |       |

<sup>(1)</sup>Oleyl Hydroxamic Acid

\*Base fuel was 190 proof ethanol.

In two separate tests, the test fuel without any additive gave scar diameters of 0.89 and 0.90 mm, respectively. The addition to the base fuel of oleyl hydroxamic acid at a concentration of 1.0 weight percent significantly reduced the wear index to 0.44 mm. Thus, the incorporation of N-hydroxy hydrocarbonamides into alcohol or alcohol containing fuels significantly increases the wear inhibiting properties of these fuels. The N-hydroxy hydrocarbonamides of the present invention are also effective anti-wear agents when used in fuel compositions comprising mixtures of monohydroxy alkanols having from 1 to 5 carbon atoms and fuel oil boiling above the gasoline boiling range, i.e. a mixture of hydrocarbons boiling in the range of from about 300° F. to about 700° F. Such compositions may also contain ignition accelerators such as the organic nitrates referred to previously.

Further, the N-hydroxy hydrocarbonamides of the present invention are also effective anti-wear agents when used in diesel fuel compositions comprising a mixture of hydrocarbons boiling in the range of from about 300° F. to about 700° F. devoid of any alcohol components. Such fuel oil compositions comprise both the heavy and light diesel fuel oils which are commonly used at present as fuels in diesel motor vehicles. Such fuel compositions may also contain ignition accelerators such as organic nitrates as well as other additives such as demulsifying agents, corrosion inhibitors, antioxidants, dyes, and the like commonly used in these types of fuel compositions.

Thus, another embodiment of the present invention is an anti-wear compression ignition fuel for use in diesel engines comprising a fuel oil boiling above the gasoline range containing a wear inhibiting amount of an N-hydroxy hydrocarbonamide.

I claim:

1. As a new composition of matter, an anti-wear compression ignition fuel for use in diesel engines comprising (1) a monohydroxy alkanol having from 1 to 5 carbon atoms, and (2) a wear inhibiting amount of an N-hydroxy hydrocarbonamide having the formula

wherein R is a hydrocarbon group having a valence of n and containing from 6 to 51 carbon atoms and n is an integer from 1 to 3.

2. The composition of claim 1 wherein said monohydroxy alkanol is ethanol.

3. The composition of claim 2 wherein said N-hydroxy hydrocarbonamide is N-hydroxy oleamide.

4. The composition of claim 2 wherein said N-hydroxy hydrocarbonamide is N-hydroxy tall oil fatty acid amide.

5. The composition of claim 2 wherein said N-hydroxy hydrocarbonamide is N-hydroxy linoleamide.

6. The composition of claim 2 wherein said N-hydroxy hydrocarbonamide is N-hydroxy amide of linoleic acid dimers, trimers or mixtures thereof.

7. The composition of claim 3 containing from about 0.01 to about 2.0 weight percent N-hydroxy oleamide based on the total weight of said composition.

8. As a new composition of matter, an anti-wear compression ignition fuel for use in diesel engines comprising (1) a monohydroxy alkanol having from 1 to 5 carbon atoms, (2) an ignition accelerator, and (3) a wear inhibiting amount of an N-hydroxy hydrocarbonamide having the formula



wherein R is a hydrocarbon group having a valence of n and containing from 6 to about 51 carbon atoms and n is an integer from 1 to 3.

9. The composition of claim 8 wherein said monohydroxy alkanol is ethanol.

10. The composition of claim 8 wherein said ignition accelerator is a substituted or unsubstituted alkyl or cycloalkyl nitrate having up to 10 carbon atoms.

11. The composition of claim 8 wherein said N-hydroxy hydrocarbonamide is N-hydroxy oleamide.

12. The composition of claim 8 wherein said N-hydroxy hydrocarbonamide is N-hydroxy tall oil fatty acid amide.

13. The composition of claim 8 wherein said N-hydroxy hydrocarbonamide is N-hydroxy linoleamide.

14. The composition of claim 8 wherein said N-hydroxy hydrocarbonamide is N-hydroxy amide of linoleic acid dimers, trimers or mixtures thereof.

15. The composition of claim 9 wherein said ignition accelerator is selected from methyl nitrate, ethyl nitrate, propyl nitrate, amyl nitrates, hexyl nitrates or a mixture of primary amyl nitrates and primary hexyl nitrates.

16. The composition of claim 15 wherein said ignition accelerator is ethyl nitrate.

17. The composition of claim 15 wherein said N-hydroxy hydrocarbonamide is N-hydroxy oleamide.

18. The composition of claim 17 containing from about 0.1 to about 10.0 weight percent ignition accelerator and from about 0.01 to about 2.0 weight percent N-hydroxy oleamide based on the total weight of said composition.

19. A method for inhibiting engine wear in an internal combustion reciprocating diesel engine operating on a compression ignition fuel comprising (1) a monohydroxy alkanol having from 1 to 5 carbon atoms, (2) an ignition accelerator, and (3) a wear inhibiting amount of an N-hydroxy hydrocarbonamide having the formula



wherein R is a hydrocarbon group having a valence of n and containing from 6 to about 51 carbon atoms and n is an integer from 1 to 3, said method comprising (a) supplying to the fuel induction system of said engine compression ignition fuel, (b) inducting air into the combustion chambers of said engine, (c) compressing said air, (d) injecting said compression ignition fuel into said combustion chambers containing said compressed air, (e) igniting said compressed mixture, and (f) exhausting the resultant combustion products resulting in reduced engine wear in said engine.

20. The method of claim 19 wherein said monohydroxy alkanol is ethanol.

21. The method of claim 19 wherein said ignition 15 accelerator is a substituted or unsubstituted alkyl or cycloalkyl nitrate having up to 10 carbon atoms.

22. The method of claim 19 wherein said N-hydroxy hydrocarbonamide is N-hydroxy oleamide.

23. The method of claim 20 wherein said ignition accelerator is selected from methyl nitrate, ethyl nitrate, propyl nitrate, amyl nitrates, hexyl nitrates or a mixture of primary amyl nitrates and primary hexyl nitrates.

24. The method of claim 23 wherein said ignition 25 accelerator is ethyl nitrate.

25. The method of claim 23 wherein said N-hydroxy hydrocarbonamide is N-hydroxy oleamide.

26. The method of claim 25 wherein said ignition accelerator is present in an amount of from about 0.1 weight percent to about 10.0 weight percent based on the total weight of said composition and said N-hydroxy oleamide is present in an amount of from about 0.01 to about 2.0 weight percent based on the total weight of the composition.

27. A method for preparing a compression ignition fuel adapted for use in diesel engines having anti-wear properties which comprises blending (1) a wear inhibiting amount of an N-hydroxy hydrocarbonamide having 30 the formula



wherein R is a hydrocarbon group having a valence of n and containing from 6 to about 51 carbon atoms and n is an integer from 1 to 3, with (2) a monohydroxy alkanol having from 1 to 5 carbon atoms, and (3) an ignition accelerator.

28. The method of claim 27 wherein said monohydroxy alkanol is ethanol.

29. The method of claim 27 wherein said ignition accelerator is a substituted or unsubstituted alkyl or cycloalkyl nitrate having up to 10 carbon atoms.

30. The method of claim 27 wherein said N-hydroxy hydrocarbonamide is N-hydroxy oleamide.

31. The method of claim 28 wherein said ignition accelerator is selected from methyl nitrate, ethyl nitrate, propyl nitrate, amyl nitrates, hexyl nitrates or a mixture of primary amyl nitrates and primary hexyl nitrates.

32. The method of claim 31 wherein said ignition accelerator is ethyl nitrate.

33. The method of claim 31 wherein said N-hydroxy hydrocarbonamide is N-hydroxy oleamide.

34. The method of claim 33 wherein said ignition accelerator is present in an amount of from about 0.1 to about 10.0 weight percent based on the total weight of said composition and said N-hydroxy oleamide is present in an amount of from about 0.01 to about 2.0 weight percent.

35. An anti-wear compression ignition fuel for use in diesel engines comprising a fuel oil boiling above the gasoline range containing a wear inhibiting amount of an N-hydroxy hydrocarbonamide having the formula



wherein R is a hydrocarbon group having a valence of n and containing from 6 to about 51 carbon atoms and n is an integer from 1 to 3.

36. The compression ignition fuel of claim 35 wherein said N-hydroxy hydrocarbonamide is N-hydroxy oleamide.

37. The compression ignition fuel of claim 35 said N-hydroxy hydrocarbonamide is N-hydroxy tall oil fatty acid amide.

38. The compression ignition fuel of claim 35 wherein said N-hydroxy hydrocarbonamide is N-hydroxy linoleamide.

39. The compression ignition fuel of claim 35 wherein said N-hydroxy hydrocarbonamide is N-hydroxy amide of linoleic acid dimers, trimers or mixtures thereof.

40. The compression ignition fuel of claim 35 containing as an ignition accelerator a substituted or unsubstituted alkyl or cycloalkyl nitrate having up to about 10 carbon atoms.

41. The compression ignition fuel of claim 36 containing an ignition accelerator selected from methyl nitrate, ethyl nitrate, propyl nitrate, amyl nitrates, hexyl nitrates or a mixture of primary amyl nitrates and primary hexyl nitrates.

\* \* \* \* \*